

## UNITED STATES PATENT OFFICE.

DANIEL H. MELOCHE, OF DETROIT, MICHIGAN, ASSIGNOR TO EARL HOLLEY, OF DETROIT, MICHIGAN.

## CORE COATING.

No Drawing.

Application filed December 26, 1922. Serial No. 609,146.

*To all whom it may concern:*

Be it known that I, DANIEL H. MELOCHE, a citizen of the United States, residing at 2241 Gladstone Ave., Detroit, in the county of Wayne and State of Michigan, have invented certain new and useful Improvements in Core Coatings, of which the following is a specification.

This invention relates to means for protecting the surface of dry sand cores from the erosive action of molten cast iron. This invention is particularly adapted for use in conjunction with permanent iron molds in which grey iron castings are made. The coating consists of an inert insulating refractory, for example magnesium oxide, suspended in water to which a little glutrin is added. The exact proportions which I have found most satisfactory for small cores approximately 1" in diameter is to mix four ounces of magnesium oxide to a gallon of water containing 5% by volume of glutrin.

The dry sand cores are merely dipped into this mixture and on being withdrawn the magnesium oxide, by reason of the presence of the glutrin, forms an adherent coating on the surface of the dry sand core. These cores are then heated in a core oven so as to thoroughly dry the coating. The magnesium oxide, by reason of its excellent refractory and insulating qualities, forms a protective coating whereby particles of the sand core are not dislodged and carried into the casting as is the case where less refractory and less insulating coatings are provided. The magnesium oxide is obtained as an im-

palpable powder known as "magnesium oxide-light."

The use of the glutrin renders the coating of magnesium oxide firmly adherent, hence the cores can be handled without the coating coming off and an intact coating is presented to the molten iron when it is poured around the core.

When a coating of silica is used in place of magnesium oxide the coating of silica fuses under the erosive action of highly heated molten iron.

If fire clay is used the coating is not sufficiently porous and the coating of fire clay prevents the core acting as a vent. The peculiar advantages of magnesium oxide are that it is not only a refractory insulator but it also provides a porous coating which will not interfere with the core acting as a vent.

This application is based upon my co-pending application, Serial No. 548,475, filed March 31, 1922.

What I claim is:

1. An insulating refractory wash for coating dry sand cores consisting of a small quantity of light magnesium oxide powder suspended in water containing a small quantity of glutrin.

2. An insulating refractory wash for coating dry sand cores consisting of an inert refractory powder suspended in water containing a small percentage of glutrin to act as a binder.

In testimony whereof I affix my signature.

DANIEL H. MELOCHE.